

(No Model.)

G. W. ENDEBROCK.

HUB BAND.

No. 289,339.

Patented Nov. 27, 1883.



Attest  
Carl Spengel  
Geo. W. Endebrock

Inventor  
George W. Endebrock  
by Knight Bros. Atty's.

# UNITED STATES PATENT OFFICE.

GEORGE W. ENDEBROCK, OF CINCINNATI, OHIO.

## HUB-BAND.

SPECIFICATION forming part of Letters Patent No. 289,339, dated November 27, 1882.

Application filed July 5, 1883. (No model.)

*To all whom it may concern:*

Be it known that I, GEORGE W. ENDEBROCK, of Cincinnati, Hamilton county, Ohio, have invented a new and useful Improvement 5 in Hub-Bands for Vehicle-Wheels, of which the following is a specification.

My invention relates to that class of hub-bands for vehicles whose muzzle is lined with gold or other fine metal.

10 My improved hub-band preferably tapers inwardly at the muzzle to a shoulder, and is usually made of malleable cast-iron.

To carry out my improvement, the hub-band is immersed, point downward, in molten tin 15 or like fusible metal, so as to fill up the pores, and at the same time to present a metallic surface such as has affinity for the finer metal, which latter is then deposited, in any desired thickness, by the electroplating process.

In the accompanying drawings, A represents in profile a portion of a vehicle-hub.

20 B represents, by axial section, a malleable-iron hub-band; b, the mouth or muzzle, the same being so formed interiorly as to taper inwardly from its front edge to a thick rib or shoulder in the manner shown, so as, without

giving the band a clumsy appearance, to greatly strengthen and stiffen it where most needed, and so as, at the same time, to present the highly-ornamental gilt, silvered, or nickel-coated interior conspicuously to view. 30 The melted tin is deposited on the band from its outer lip as far back as its shoulder, so as to close the pores of the band and provide metallic surface of a kind that will receive and retain the lamina C, of silver or other fine metal, deposited. Where desired, I apply tin plating and gold, silver, brass, or nickel coating to the outside also of the band. 35

This manufacture entirely dispenses with the customary costly processes of grinding and finishing prior to coating or plating.

Having thus described my invention, I claim as new and of my invention—

40 A hub-band having a coating of melted tin on the interior of the muzzle overlaid with a coating of fine metal, as set forth.

In testimony of which invention I hereunto set my hand.

GEORGE W. ENDEBROCK.

Witnesses:

CARL SPENGEL,  
S. S. CARPENTER.